

# UNITED STATES PATENT OFFICE.

OTTOKAR SERPEK, OF PARIS, FRANCE, ASSIGNOR TO SOCIÉTÉ GÉNÉRALE DES  
NITRURÉS, OF PARIS, FRANCE.

## PROCESS OF FIXING NITROGEN.

1,155,840.

Specification of Letters Patent.

Patented Oct. 5, 1915.

No Drawing.

Application filed December 23, 1913. Serial No. 808,478.

*To all whom it may concern:*

Be it known that I, OTTOKAR SERPEK, a subject of the Emperor of Austria-Hungary, and a resident of 12 Rue Roqueline, Paris, 5 France, have invented a new and useful Process of Fixing Nitrogen, of which the following is a specification.

It is known that when ferro-aluminium is converted into nitrid, (1) the reaction takes 10 place at a relatively low temperature compared with those in use in the manufacture of aluminium nitrid when starting from ores of aluminium, and (2) the reaction is exothermic. This being admitted, the present 15 invention is based upon the following observations:—It has been found that the evolution of heat is sufficient to raise the temperature of the mass which has been previously heated to about 1200° C., up to or even 20 beyond 1900° C. Moreover, there has been ascertained the extremely surprising fact that by operating in the same way with a ferro-aluminium to which has been added a mixture of bauxite and carbon, this addition, 25 far from hindering the rise of temperature, allows of obtaining temperatures at least as high if not actually higher, that is to say such that a reaction of the nitrogen upon the mixture of bauxite and carbon can 30 take place, and that further there is obtained an improved fixation of nitrogen upon the ferro-aluminiums, even so far as to obtain in certain cases a fixation of nitrogen corresponding to the whole of the aluminium contained in the mass. 35

The process of the present invention consists therefore in passing a current of nitrogen over a mixture of ferro-aluminium, bauxite, or other aluminous materials and 40 carbon, raised to comparatively low temperatures.

Example: About 100 kilograms of finely pulverized ferro-aluminium, containing 45 per cent. of aluminium, are heated to 1200— 45 1300° in a crucible with 18 kilograms of bauxite and 7 kilograms of carbon. The temperature of the mass rises from 1200° to about 1850° and then falls slowly, remaining for five hours above 1500° C.

The process is likewise applicable to the fixation of nitrogen by means of ferro compounds other than ferro-aluminium, in which compounds the body combined with the iron is capable of fixing nitrogen; this fixation is carried out by adding to these 55 compounds a mixture of carbon and the oxid of the element combined with the iron. For example ferro-silicon may be treated with nitrogen in presence of silica and carbon; ferro-boron in presence of boric acid and 60 carbon and so on, the different oxids with the carbon being intimately mixed with the ferro compound or arranged at one or more points in the mass of the same.

There may likewise be obtained complex 65 nitrids by treating a ferro compound to which have been added carbon and an oxid of a body other than that which is combined with the iron. For example, one may treat a mixture of ferro-aluminium, silica and 70 carbon, and so on.

It is evident that the process is likewise applicable to the conversion into nitrids of complex ferro compounds in presence of mixtures of carbon and of one or more oxids 75 capable of fixing nitrogen.

In the following claims I use the expression "aluminous material" in a sufficiently general sense to embrace either alumina or substances such as bauxite, kaolin or the like; and the nitrogen may be either pure nitrogen or a gaseous body containing it.

I claim as my invention:—

1. A process of fixing nitrogen, consisting in subjecting ferro-aluminium to the action 85 of nitrogen in the presence of a mixture of carbon and aluminous material, heating to the temperature of fixation of nitrogen on the ferro-aluminium, and allowing the temperature to rise, by the exothermic reaction, 90 to the temperature of fixation of nitrogen on the aluminium of the aluminous material mixed with carbon.

2. A process of fixing nitrogen, consisting in subjecting ferro-aluminium to the action 95 of nitrogen in the presence of a mixture of carbon and aluminous material, heating to about 1200° C. and allowing the tempera-

ture to rise, by the exothermic reaction of the nitrogen on the ferro-aluminium, up to about 1800°-1900° C. a temperature at which the fixation of nitrogen on the aluminium of the aluminous material mixed with carbon is produced.

In testimony whereof I have signed my

name to this specification, in the presence of two subscribing witnesses.

**OTTOKAR SERPEK.**

Witnesses:

HANSON C. COXE,  
LÉON PEILLET.

**Copies of this patent may be obtained for five cents each, by addressing the "Commissioner of Patents, Washington, D. C."**